

# UNITED STATES PATENT OFFICE.

JOHN GAST, OF BROOKLYN, NEW YORK.

## VULCANIZED-RUBBER PAD FOR STIGMOGRAPHS.

SPECIFICATION forming part of Letters Patent No. 242,627, dated June 7, 1881.

Application filed March 25, 1881. (No model.)

*To all whom it may concern:*

Be it known that I, JOHN GAST, of Brooklyn, in the county of Kings and State of New York, have invented a new and useful Improvement in Vulcanized-Rubber Pads for Stigmographs, of which the following is a specification.

The invention relates to an improved pad for stippling on lithographic stones, zinc or metal plates, and for other uses in the art of lithography.

The object of the invention is to produce a pad whereby stipple-work may be rapidly and artistically accomplished, and which will be of such elasticity that it will yield sufficiently to pressure, and which will be of the necessary durability, and neither shrink, break, nor crack when subjected to ordinary atmospheric changes. I have termed the pad mentioned a "stigmograph," by which it will be described hereinafter.

The following is a formula of the ingredients constituting the preferred composition out of which the stigmograph is made: Ten (10) pounds of rubber; twelve (12) ounces of sulphur; forty-eight (48) ounces of vermillion; twenty (20) ounces of French zinc-white; four (4) ounces of powdered soapstone. These ingredients are thoroughly mixed together, gentle heat being applied to render the mass homogeneous.

While a compound consisting of the above-named ingredients is preferred for the formation of the stigmograph, it is plain that they may be varied somewhat without departing from the essence of the invention. For instance, in lieu of employing vermillion, which gives the compound a reddish color, I may use an analogous material. If a yellow color is to be produced, I employ chrome-yellow and cadmium; if a green color, I use chrome-yellow or lemon-yellow and Antwerp blue, Prussian, Milori, or any other blue. For a blue color I prefer to use chrome-green and ultramarine or cobalt. It will be desirable, however, to employ a color of about the same relative weight and bulk as vermillion to attain the proper degree of elasticity. If the color used is much lighter in weight than vermillion, its proportion of weight should be made up with the zinc-white or its equivalent. The compound is now in one homogeneous mass, and my object is to re-

duce it to small pieces or pads of proper size and thickness, one side of the same being smooth and the other side having a stippled or grained surface in relief, the piece or pad being also vulcanized.

The process of treating the compound to form the pads described will be as follows: I first draw or stipple on stone with pen the style and size of grain of stipple-work to be produced in relief on the surface of the pad or stigmograph. Of course the size and style of grain may be varied at will. From the stone a print of the stipple-work is taken on white paper, from which relief-plates are made by the photo-engraving process or any other suitable method. I next take plaster casts or negative metal casts from the relief-plates, and from these plaster or metal casts the rubber pads or stigmographs receive the impression of the stipple-work. The pads, having been thus formed, are then vulcanized according to the following method: The rubber compound is rolled into a thin sheet of, say, about one-eighth of an inch in thickness, and then cut into smaller pieces or pads of proper size to fit the plaster negatives, (or plaster molds,) upon which they are placed and pressed firmly down by a smooth polished metallic plate applied to the back of the rubber, whereby the said back is given a smooth surface.

As a precaution, prior to placing the metal plate upon the rubber I prefer to first powder the back of the pad with fine soapstone-dust and then spread a smooth sheet of tin-foil over it, afterward placing the polished metal plate upon the tin-foil. This is done to prevent the metal from blackening the back of the pad during the vulcanization of the latter. The metal plate is screwed tightly to the plaster mold by means of a pair of clamp-irons of usual construction. In order to prevent the plaster mold from breaking during the operation, it may be formed within an iron chase of proper size. The plaster mold, with the rubber held upon its surface by the polished plate and clamp-irons, is then introduced into a steam-vulcanizer and submitted to a heat of about 265° Fahrenheit for a space of about four and one-half to five hours. I recommend that great care be exercised in this step of the process, since the proper vulcanization adds greatly in giving the pad the required toughness and

elasticity, so as to be just suitable and applicable to transfer an impression by the touch of the finger, hand, or stylus. After the vulcanization the pads are taken out and are ready 5 for use, one side being smooth and the other bearing the impression of stipple-work taken from the plaster mold.

The foregoing is an accurate description of the stigmograph and the mode of its manufacture. In using it for stippling stone the following steps should be observed: The outlines of the design being drawn, the solids filled in, and the sharp lines gummed out in the usual way, the stigmograph, which has received a 15 coating of lithographic transfer-ink from a common printer's roller or otherwise, is laid over the stone where wanted. If an even tint is desired, the instrument is pressed gently and evenly with the hand or otherwise; and if 20 a darker tint or thicker dots are required, the pressure is increased.

If it is not desired to gum out the lights on the stone, they may be scraped out, like those on what are known as "rub tints" or "asphalt drawings," and beautiful soft effects produced. 25

The stigmograph described, in lieu of being a flat printing-pad, may be mounted upon a roller or otherwise, as may be preferred.

I am aware that elastic printing-films, hand-

stamps, &c., have been long known in the arts; 30 but none of them, as far as I am informed, have possessed that peculiar degree of elasticity upon which I rely, which is essential to the production of really artistic effects, and the permanent preservation of which is necessary in 35 an instrument of practical value.

What I claim as new is—

1. A stigmograph composed of rubber, sulphur, a color, French zinc-white, and powdered soapstone, in about the proportions stated. 40

2. A stigmograph formed from a sheet consisting of rubber, sulphur, a color, French zinc-white, and powdered soapstone, and vulcanized.

3. A stigmograph consisting of a sheet formed 45 from a rubber compound and vulcanized by being subjected to a heat of about 265° Fahrenheit for a space of from about four and one-half to five hours, substantially as set forth.

In testimony that I claim the foregoing improvement in vulcanized-rubber pads, as above described, I have hereunto set my hand this 24th day of March, 1881.

JOHN GAST.

Witnesses:

JOHN T. FINN,

HARRY C. DOYLE.